

# UNITED STATES PATENT OFFICE.

GUILLIAM H. CLAMER, OF PHILADELPHIA, PENNSYLVANIA.

## PROCESS OF MAKING AN IRON-NICKEL-COPPER ALLOY.

1,086,314.

Specification of Letters Patent.

Patented Feb. 3, 1914.

No Drawing.

Application filed July 21, 1910. Serial No. 573,094.

*To all whom it may concern:*

Be it known that I, GUILLIAM H. CLAMER, a citizen of the United States, residing at Philadelphia, in the county of Philadelphia 5 and State of Pennsylvania, have invented a certain new and useful Process of Making an Iron-Nickel-Copper Alloy, of which the following is a specification.

In my application for Letters Patent of 10 the United States, serially numbered 513,537, I have described and claimed what I call a high range nickel-copper-iron alloy, and which can be made within the following range of proportions by weight: nickel 25 15 to 50, copper 5 to 20, iron 30 to 70, together with a small amount of impurities such as would ordinarily exist in commercial steel, copper and nickel.

In my application serially numbered 20 513,538, filed August 19th, 1909, I have described a process for producing iron-copper-nickel alloys direct from ore containing nickel and copper and iron in the form of sulfids, and in that application have referred to the high range alloy. In my application serially numbered 573,095 filed 25 July 21st 1910, I have described and claimed what I call low range alloys of copper, iron and nickel, which contain iron, nickel up to 30 6 per cent., and copper up to two per cent., from, for example, a half of 1 per cent.

The present invention has to do with the use of Monel metal in the production of alloys of both the high and low ranges, and 35 also with the production of the low range alloy direct from ore containing nickel and copper and iron in the form of sulfids, and the object of the present invention is to provide an expeditious and economical method 40 of producing alloys of both the high and low ranges.

It may be stated that steels between the ranges given are hard and brittle and of no commercial value, and are of "Martensitic" 45 structure, whereas those of high range have a crystalline structure and those of low range a pearlitic structure. Since copper is cheaper than nickel, it is evident that an economy is effected by replacing nickel with 50 copper, and this can be accomplished with-

out diminishing the desirable properties of the metal, and in fact, with some increase of those desirable properties. To make the low range alloy directly from ore containing nickel, copper and iron in the form of sulfids, the ore is first melted with fluxes to form a slag with the gangue, and the production at the same time of an iron-copper-nickel matte. This matte may be of varying composition. This matte is then calcined 55 to remove sulfur and convert the nickel, copper and iron into oxids. These oxids are reduced with carbon or other suitable reducing agent, whereby there is produced a homogeneous alloy of the three metals in substantially relative proportions in which they exist in the matte before calcining. In the reducing operation if carbon and impurities are introduced in excessive amounts they may be removed to the extent desired by any 60 of the well-known oxidizing processes used in steel making. The addition of any of the three metals, copper, nickel or iron, may be made to bring the alloy to the desired proportions, but where the ores contain the metals in the proper proportions this addition is, of course, unnecessary.

In the manufacture of both the high and low range alloys or nickel steels containing copper in the proportions set forth, use may be made of Monel metal. Monel metal is an alloy of approximately 68 per cent. nickel, 2 per cent. iron and 30 per cent. copper, and in accordance with my invention is added to iron in the proper proportions, and when Monel metal is used the double melting is advantageous, because it improves the uniformity of the product. Monel metal, as is well known, can be made directly from ore containing nickel, copper and iron in the form of sulfids by first melting the ore with fluxes to form a slag with the gangue, and produce an iron-copper-nickel matte, then bessemerizing this matte to remove as much iron as is possible, which is all except about 95 2 per cent., and then calcining the matte to remove sulfur and convert the nickel, copper and iron into oxids which are reduced with carbon or other suitable reducing agent.

What I claim is:

The method of making an iron-nickel-copper alloy which consists in making an iron-copper-nickel matte from sulfid ore containing iron, copper and nickel, calcining the matte to convert the sulfid of iron, nickel and copper into oxids, reducing the oxids thereby making an alloy of the metals named con-

taining all the iron of the original ore and eliminating carbon and impurities to the extent desired.

GUILLIAM H. CLAMER.

Witnesses:

S. E. PATTERSON,  
K. M. GILLIGAN.